

## UNITED STATES PATENT OFFICE

2,176,942

## ABRASIVE IMPLEMENT

Lawrence V. Redman, Caldwell, N. J., assignor,  
by mesne assignments, to Behr-Manning Cor-  
poration, Troy, N. Y., a corporation of Massa-  
chusetts

No Drawing. Application August 19, 1927,  
Serial No. 214,219

6 Claims. (Cl. 51—280)

This invention relates to abrasive implements, and comprises a novel implement of this character wherein the abrasive grains (silicon carbide, crystalline alumina, emery, sand, etc.) are bonded by an infusible but non-rigid or flexible bonding agent, which for purposes of identification I will term a "flexible phenolic resin". The term "abrasive implement" is used broadly herein to include not only abrasive sheets, discs and other 5 grinding and cutting tools, but also polishing wheels or discs, emery and sand papers and cloths and the like. It is in these last-mentioned applications, where the abrasive grain is applied to a flexible base such as paper, cloth or felt, that 10 the advantages of my invention are most strikingly exhibited.

Infusible and insoluble resins of the well known phenol-aldehyde type have long been used for bonding abrasive grains for making grinding 15 wheels and other implements. This is disclosed for example in United States Patent 942,808 to L. H. Baekeland, and United States Patent 1,537,454 to Brock. In these cases, however, and in all prior cases of which I am aware wherein 20 resins of the phenol-aldehyde type have been used, the object has been to provide a strong, hard, infusible, rigid bond for the grains unless modified by high boiling solvents or plasticizers as disclosed in a prior patent to Baekeland 25 1,019,407, March 5, 1912, or my prior Patent 1,107,703, August 18, 1914. Both of these patents describe glycerine and similar modifying agents but plasticizers of this nature have a tendency 30 to reduce the strength or adhesion of the bond to the grains in proportion to the amount of plasticizer included and to cause the resin binder to exhibit an increase in plasticity with a rise in 35 temperature. According to the present invention, on the contrary, I provide an inherently non-rigid or flexible but infusible bond, which not only permits some freedom of movement to the 40 bonded grains when subjected to strain or pressure, but allows these grains to be affixed to such flexible bases as cloth, paper or felt. At the same time, for reasons which insofar as they are understood are explained below, the resulting implements retain to a remarkable degree their 45 initial free-cutting character, as compared with like implements in which the grains are bonded by glue or other substance which melts or softens 50 to a "tacky" state at the working temperature.

It is well known that abrasive papers and cloths as heretofore available, rather quickly lose their free-cutting characteristics in use. 55 This is due to several causes among which are the following:

1. Under the very considerable rise of temperature due to the friction between the abrasive and the work and the cutting action of the abrasive, the usual bonds soften and flow, coating the grains.

2. Under the same conditions these bonds become "tacky", and pick up and tenaciously hold both the abrasive dust and the dust from the work, with the result that the interstices between the grains are soon partly or completely filled, 10 and the initial free-cutting character is lost.

I have found that both of these difficulties can be overcome by providing a bond which, although initially flexible, does not fuse nor become tacky at any temperature to which the implement is 15 subjected in use. So far as I am aware no bond having these essential characteristics has been applied heretofore in the manufacture of abrasive implements. Prior bonding materials have either been initially rigid, in which case they 20 could not be applied with advantage to flexible bases; or if initially flexible they have softened unduly under working conditions.

I have found that certain flexible phenolic resins, heretofore used as coating compositions, 25 possess to a very remarkable degree the desirable qualities above indicated; and that when used for bonding abrasive grains in the manufacture of abrasive papers and cloths they yield a product characterized in marked degree by freedom from 30 tendency to fill and clog. While my invention is not limited to a particular composition of binder I prefer to use for the purpose such flexible phenolic resins as may be prepared, for example, by effecting a reaction between tung oil and 35 phenol in presence of a converting agent or catalyst, and further hardening the resulting phenolic complex to its ultimate infusible state with hexamethylenetetramine or other methylene-containing or aldehyde hardening agent 40 and sufficient application of heat. For example resinous compositions well adapted for the present purpose may be prepared as described in United States Patent 1,590,079 to Byck. But as stated above my invention is not restricted to the 45 use of this particular composition, but contemplates the employment of any equivalent composition possessing the essential qualities of flexibility at normal as well as higher temperatures, joined with freedom from any substantial tendency to fuse or become tacky at the highest 50 temperatures developed during use.

A further and very advantageous application of these flexible bonding agents is in the manufacture of polishing implements. If a rigid bond 55 is used such abrasive grains as project beyond

the rest tend to cut or scratch the work; whereas with the flexible bond such projecting grains yield to the pressure, and a true polishing effect is obtained. The polishing implement may assume various forms according to the character of work to be done. For example it may consist of an assembly of fabric discs, mounted on a central shaft, and each coated around the peripheral portion with the abrasive grains, flexibly bonded as above described. Or it may comprise a metallic or other disc, rotatably mounted, and provided with a heavy felt rim which carries the flexibly bonded abrasive. These polishing implements, like the abrading and cutting tools described above, retain to a remarkable degree their efficiency and free-working characteristics, owing as already explained to the non-flowing character of the bond, and its freedom from tackiness at high temperatures, coupled with a high degree of flexibility at all temperatures.

The above-described flexible phenolic resins possess other advantages. Thus they are unaffected by water or oil, and resistant to most chemicals, to air-oxidation, and to all common solvents. These qualities they possess in common with the resinoids of the phenol-aldehyde type which have long been used for bonding abrasives. Like the phenolaldehyde resinoids they are infusible at any temperature. But unlike these resinoids they are highly flexible, and hence adapted for such abrading, cutting and polishing purposes as require their attachment to a flexible base or carrier.

I claim:

1. As a new article of manufacture, an abrasive implement comprising a flexible base, abrasive grains, and a binder for securing said grains to said base, said binder including the reaction prod-

uct of a phenol with oil and a methylene-containing agent, and characterized by inherent flexibility and insolubility.

2. As a new article of manufacture, an abrasive implement comprising a flexible base, abrasive grains, and a binder for securing said grains to said base, said binder including a phenol-oil resin reaction product.

3. An abrasive article comprising an undistorted composite of a sheet of cellulosic backing material and a grit or layer of abrasive particles and a binder uniting said particles to the backing comprising the polymerized reaction product of a fatty oil, a phenol and substance having an active methylene group soluble in the oil.

4. An abrasive article in the nature of sandpaper comprising a composite of a sheet of cellulosic backing material and a grit or layer of abrasive particles and a binder uniting said particles to the backing comprising the polymerized and oxidized reaction product of a fatty oil, a phenol and a substance having an active methylene group soluble in the oil.

5. An abrasive article comprising a composite of a sheet of cellulosic backing material and a layer of abrasive particles and a binder uniting said particles to the backing comprising the polymerized reaction product of a fatty oil, a phenol and substance having an active methylene group.

6. An abrasive article in the nature of sandpaper comprising a composite of a sheet of cellulosic backing material and a layer of abrasive particles and a binder uniting said particles to the backing comprising the polymerized and oxidized reaction product of a fatty oil, a phenol and a substance having an active methylene group.

LAWRENCE V. REDMAN.